# EUROPEAN PATENT SPECIFICATION

(11) **EP 0 233 058 B1**
(45) Date of publication and mention of the grant of the patent: **06.11.1991**
(21) Application number: 87301007.8
(22) Date of filing: 05.02.1987
(51) Int. Cl.: D21F 11/04

(54) **Method and apparatus of manufacturing multilayer board**
Verfahren und Einrichtung zur Herstellung von mehrschichtigem Karton
Procédé et appareil pour la fabrication d'un carton multicouche

(30) Priority: 11.02.1986 FI 860606
(43) Date of publication of application: 19.08.1987
(73) Proprietor: Valmet-Karhula Inc., 48601 Karhula (FI)
(72) Inventor: Waris, Tapio, SF-47800 Kyminlinna (FI)
(74) Representative: Gilmour, David Cedric Franklyn

(56) References cited:
- EP-A- 0 109 282
- WO-A-85/05387
- DE-A- 2 310 445
- DE-B- 1 136 198
- GB-A- 2 041 030
- US-A- 2 286 942
- US-A- 4 021 295

## Description

The present invention relates to a method of manufacturing a multilayer board web, wherein superposed pulp layers are formed by headboxes disposed on a fourdrinier wire with two intermediate headboxes feeding intermediate high consistency stock layers being fed between two surface layers formed by headboxes providing low consistency stock layers; and wherein the consistency of the high consistency stock layers is so high that, in a slice channel of the intermediate headboxes or after the stock has been discharged from each intermediate headbox slice, the forming pulp layers reach such a degree of felting that the fibres of the pulp cannot significantly move on the wire in relation to one another, and that dewatering of the high consistency layers takes place through the wire, and to an apparatus therefor.

When manufacturing multilayer boards, layers of different qualities are used. The core layer that gives sturdiness and rigidity to the board is often manufactured from pulps made of waste paper, whilst the surface layers or at least one surface layer is usually made from bleached pulp of better quality.

With multilayer board machines in which several pulp layers are bonded by wet pressing, a strong and rigid packaging board that has good printing qualities and a grammage of 200-600 g/m² can be produced with low costs for raw materials.

A very old method of manufacturing multilayer board involves manufacturing the layers with cylinder moulds. The driving speed of cylinder moulds is, however, relatively slow and high stock consistencies cannot be used in them which thus involves large dewatering quantities. In addition, a plurality of cylinder moulds are needed if the board is required to be very thick.

Fourdrinier wire machines can be driven at higher speeds than cylinder moulds and the sheet formation can be better controlled in them. Multiwire fourdrinier machines are most suitable when manufacturing thin board qualities. High investment and running costs, however, limit the use of these machines.

In the closest known prior art WO 85/05387 of A. Ahlstrom Corporation there is disclosed a method for manufacturing multilayer board in which the pulp suspension forming a surface layer 12 is fed onto the horizontal section of a first, inner wire 1. The pulp suspension forming an intermediate layer 11 is supplied onto said web layer, which is already formed, in or in front of a tapering gap 6 constituted by the first wire and a second, outer wire 4. Both of the wires and the web layers 11, 12 between them are guided over a curved surface 3. After this the first wire and both of the web layers are guided against a third, lower wire 8 onto the horizontal section of which the pulp suspension forming the other surface layer 13 is supplied. The consistency of the pulp suspension forming the intermediate layer 11 is higher than that of the pulp suspensions forming the surface layers. Mention is made on page 4 of this document of the possibility of the provision of a fourth headbox between the turning roll 7 and the headbox 14 on the lower wire 8 (or the headboxes 9 and 10) to supply another intermediate layer on the horizontal section of the lower wire 8 although the nature of the fourth headbox is not specifically mentioned. In this arrangement the formation of one or two layers on a lower wire 8 naturally requires apparatus for such and consequentially has a greater space requirement in the lower region of the apparatus.

The main object of the present invention is to provide a method of manufacturing high grammage (500 - 700 g/m²) multilayer board with simple means. This is achieved according to the present invention by the provision of a method of manufacturing a multilayer board web, wherein superposed pulp layers are formed by headboxes disposed on a fourdrinier wire with two intermediate headboxes feeding intermediate high consistency stock layers being fed between two surface layers formed by headboxes providing low consistency stock layers; and wherein the consistency of the high consistency stock layers is so high that, in a slice channel of the intermediate headboxes or after the stock has been discharged from each intermediate headbox slice, the forming pulp layers reach such a degree of felting that the fibres of the pulp cannot significantly move on the wire in relation to one another, and that dewatering of the high consistency layers takes place through the wire; wherein the pulp layers are formed on a single wire, and the formed pulp layers between the two intermediate high consistency headboxes is smoothed by a dandy roll.

Also according to the present invention there is provided an apparatus for manufacturing a multilayer board according to the method of claim 1, wherein headboxes are disposed on a fourdrinier wire for forming superposed pulp layers with two of the headboxes being provided to form two surface layers formed from low consistency stock and with two of the headboxes being intermediate headboxes for feeding intermediate high consistency stock layers between said two surface layers, wherein the two intermediate headboxes are such that the stock consistency supplied thereby is so high that, in a slice channel of the intermediate headboxes or after the stock has been discharged from each intermediate headbox slice, the forming pulp layers reach such a degree of felting that the fibres of the pulp cannot significantly move on the wire in relation to one another, and that dewatering of the high consistency layers takes place through the wire; and wherein a single wire is provided for the formation of the superposed layers, and a dandy roll is provided between the two intermediate high consistency headboxes to act to smooth the formed pulp layer between said headboxes.

The invention will be described further, by way of example, with reference to the accompanying drawing which is a schematic illustration of a section of a web forming section in a board machine according to the invention.

A web forming section of a board machine is illustrated in Fig. 1 and is a twin wire former comprising a first wire arrangement or first wire 1 having a main run which generally extends horizontally from a breast roll 2 to a forming roll 3 and a second wire arrangement or wire 4 which forms with the first wire a gap 5 that tapers towards the forming roll. After the forming roll 3 both wires run diagonally downwards and the second wire 4 is detached from the first wire. Under the horizontal section of the first wire 1 are disposed known (not shown), wire supporting dewatering devices such as vacuum boxes and foils which effect dewatering downwardly through the wire.

The stock forming the first outer ply of the board is fed onto the first wire 1 by a headbox 6 which is disposed at the breast roll 2 and operates at a normal consistency range of 0.1 to 1.2%.

The layers forming the core of the multilayer board are produced by feeding stock onto the wire on top of the already formed web layer by two intermediate high consistency headboxes 7 and 8 disposed at a distance from each other in which the stock consistency is substantially higher than the normal headbox consistency, e.g. 3%.

A headbox of this type is described in e.g. Finnish Patent Publication No. 56221. When the slice spray reaches the wire at this consistency, the drainage of the pulp does not take place in the same way as at a normal headbox consistency, but rather the web is formed in such a way that the fibres form a continuous network across the whole thickness of the web in the slice channel of the headbox or immediately after it. The web structure becomes felted and there is a relatively strong z-orientation of the fibres in the web. The structure of a web formed at a normal consistency is on the contrary stratified. During the web formation the felted structure remains more open than the stratified structure which means that dewatering of such a web is easier than that of a web formed at a normal consistency which again makes it possible to drain water from the pulp layer formed by the headbox 8 downwards through the pulp layer formed by the headbox 7. Since the quantity of water to be drained from the pulp layers is considerably smaller than that to be drained from pulp layers formed at a normal consistency, both layers can be thick and a thick core can be produced by two headboxes. Due to the fibre orientation, the core also has a higher bulk than a core formed at a normal consistency.

The web formation of a multilayer board can be improved by treating the web by means of a dandy roll 9 disposed between the headboxes 7 and 8.

The second thin outer ply is supplied by a headbox 10 which is disposed in front of the gap formed by the first and second wires 1 and 4 and which operates at a normal consistency range. The web layers on the forming roll 3 are pressed between the wires 1 and 4 and due to the centrifugal force water is drained upwards through the wire 4. Subsequently the thus formed 4-ply web is guided by known methods to the press and dryer sections of a board manufacturing machine for further treatment.

The stock consistency in the high consistency headboxes 7 and 8 is 1.5 - 6% or higher, preferably 2 - 4%. The grammage of the core layers formed at a high consistency can be 100 - 300 g/m² or higher, preferably 150 - 250 g/m². Thus a 4-ply board with a grammage of ca. 600 g/m² can be manufactured on a relatively short twin wire former.

The invention is not only limited to the described embodiment presented as example, but several modifications and applications may be made of it within the scope of the invention concept defined by the appended claims.

It will be understood by persons skilled in the art that the term "fourdrinier wire" throughout the specification and claims, relates to and is generally understood to mean an endless belt arrangement as is used in fourdrinier machines which is sometimes referred to as a "cloth" and which may, e.g. be made of a wire mesh (mesh of metal filaments) or of a plastics material mesh.

## Claims

1. A method of manufacturing a multilayer board web, wherein superposed pulp layers are formed by headboxes disposed on a fourdrinier wire with two intermediate headboxes feeding intermediate high consistency stock layers being fed between two surface layers formed by headboxes providing low consistency stock layers; and wherein the consistency of the high consistency stock layers is so high that, in a slice channel of the intermediate headboxes or after the stock has been discharged from each intermediate headbox slice, the forming pulp layers reach such a degree of felting that the fibres of the pulp cannot significantly move on the wire in relation to one another, and that dewatering of the high consistency layers takes place through the wire, wherein the pulp layers are formed on a single wire, and the formed pulp layer between the two intermediate high consistency headboxes is smoothed by a dandy roll.

2. A method according to claim 1 characterised in that the stock consistency is 2 - 4%.

3. A method according to claims 1 or 2 characterised in that the grammage of each of the pulp layers is 100 - 300 g/m².

4. A method according to any one of claims 1 to 3 characterised in that the high consistency pulp layers form the core of the multilayer board.

5. An apparatus for manufacturing a multilayer board according to the method of claim 1, wherein headboxes (6, 7, 8, 10) are disposed on a fourdrinier wire (1) for forming superposed pulp layers with two of the headboxes (6, 10) being provided to supply two surface layers formed from low consistency stock and with two of the headboxes (7, 8) being intermediate headboxes (7, 8) for feeding intermediate high consistency stock layers between said two surface layers, wherein the two intermediate headboxes (7, 8) are such that the stock consistency supplied thereby is so high that, in a slice channel of the intermediate headboxes (7, 8) or after the stock has been discharged from each intermediate headbox slice, the forming pulp layers reach such a degree of felting that the fibres of the pulp cannot significantly move on the wire (1) in relation to one another, and that dewatering of the high consistency layers takes place through the wire; and wherein a single wire (1) is provided for the support of the superposed layers, and a dandy roll (9) is provided between the two intermediate high consistency headboxes (7, 8) to act to smooth the formed pulp layer between said headboxes (7, 8).

## Revendications

1. Procédé de fabrication d'une nappe de carton multicouches, dans laquelle des couches de pulpe superposées sont formées par des caisses de tête disposées sur une toile de fourdrinier avec deux caisses de tête intermédiaires fournissant des couches de matériau de consistance élevée qui sont amenées entre deux couches de surface formées par les caisses de tête fournissant des couches de matériau de faible consistance ; et dans lequel la consistance des couches de matériau de consistance élevée est si élevée que, dans une conduite à segments des caisses de tête intermédiaires ou quand le matériau a été déchargé de chaque tranche de caisse intermédiaire, les couches de pulpe en formation atteignent un tel degré de feutrage que les fibres de la pulpe ne peuvent pas se déplacer de façon significative sur la toile par rapport l'une à l'autre, et qu'une déshydratation des couches de consistance élevée se produit à travers la toile, dans lequel les couches de pulpe sont formées sur une seule toile et la couche de pulpe formée entre les deux caisses de tête intermédiaires de consistance élevée est lissée par un rouleau égoutteur.

2. Procédé selon la revendication 1 caractérisé en ce que la consistance du matériau est 2-4%.

3. Procédé selon les revendications 1 ou 2 caractérisé en ce que le grammage de chacune des couches de pulpe est de 100-300 g/m².

4. Procédé selon l'une quelconque des revendications 1 à 3 caractérisé en ce que les couches de pulpe de consistance élevée forment le coeur du carton multicouches.

5. Dispositif pour fabriquer un carton multicouches selon le procédé de la revendication 1, dans lequel des caisses de tête (6,7,8,10) sont disposées sur une toile de fourdrinier (1) pour former des couches de pulpe superposées avec deux des caisses de tête (6, 10) qui sont prévues pour approvisionner deux couches de surface formées d'un matériau de faible consistance et avec deux des caisses de tête (7,8) qui sont des caisses de tête intermédiaires (7,8) pour amener des couches intermédiaires de matériau de consistance élevée entre lesdites deux couches de surface, dans lequel les deux caisses de tête intermédiaires (7,8) sont telles que la consistance du matériau fourni par elles est si élevée que, dans une conduite à segment des caisses de tête intermédiaires (7,8) ou après que le matériau a été déchargé de chacun des segments de caisses de têtes intermédiaires, les couches de pulpe en formation atteignent un tel degré de feutrage que les fibres de la pulpe ne peuvent pas de façon significative, se déplacer sur la toile (1) l'une par rapport à l'autre, et telles qu'une déshydratation des couches de consistance élevée se produit à travers la toile; et dans lequel une seule toile (1) est prévue comme support des couches superposées, et un rouleau égoutteur (9) est prévu entre les deux caisses de tête intermédiaires de consistance élevée (7,8) pour pouvoir lisser la couche de pulpe formée entre lesdites caisse de tête (7,8).

## Patentansprüche

1. Verfahren zur Herstellung einer mehrschichtigen Pappbahn, worin übereinanderliegende Pulpeschichten durch Stoffauflaufkästen gebildet werden, die an einem Fourdrinier-Drahtnetz angeordnet sind, wobei zwei Zwischenstoffauflaufkästen Zwischenstoffschichten hoher Stoffdichte zuführen, die zwischen zwei Oberflächenschichten zugeführt werden, die durch Stoffauflaufkästen gebildet werden, die Stoffschichten niedriger Stoffdichte vorsehen; und worin die Stoffdichte der Stoffschichten hoher Stoffdichte so hoch ist, daß in einem Staukanal der Zwischenstoffauflaufkästen, oder nachdem der Stoff von jeder Stauvorrichtung der Zwischenstoffauflaufkästen abgelassen ist, die formenden Pulpeschichten einen solchen Filzgrad erreichen, daß sich die Fasern der Pulpe auf dem Drahtnetz gegeneinander nicht wesentlich bewegen können, und daß die Entwässerung der Schichten hoher Stoffdichte entlang des Drahtnetzes stattfindet, wobei die Pulpeschichten auf einem einzelnen Drahtnetz ausgebildet werden und die zwischen den beiden Zwischenstoffauflaufkästen hoher Stoffdichte ausgebildete Pulpeschicht durch eine Druckrolle geglättet wird.

2. Verfahren nach Anspruch 1,
dadurch **gekennzeichnet,** daß
die Stoffdichte 2 bis 4 % beträgt.

3. Verfahren nach Anspruch 1 oder 2,
dadurch **gekennzeichnet,** daß
das Quadratmetergewicht jeder Pulpeschicht 100 - 300 g/m² beträgt.

4. Verfahren nach einem der Ansprüche 1 bis 3,
dadurch **gekennzeichnet,** daß
die Pulpeschichten hoher Stoffdichte den Kern der mehrschichtigen Pappe bilden.

5. Vorrichtung zum Herstellen mehrschichtiger Pappe nach dem Verfahren nach Anspruch 1, bei der Stoffauflaufkästen (6, 7, 8, 10) an einem Fourdrinier-Drahtnetz (1) angeordnet sind, um übereinanderliegende Pulpeschichten auszubilden, wobei zwei der Stoffauflaufkästen (6, 10) vorgesehen sind, um zwei Oberflächenschichten zuzuführen, die aus Stoff niedriger Stoffdichte gebildet sind, und wobei zwei der Stoffauflaufkästen (7, 8) Zwischenstoffauflaufkästen (7, 8) sind, die Zwischenstoffschichten hoher Stoffdichte zwischen den beiden Oberflächenschichten zuführen, wobei die beiden Zwischenstoffauflaufkästen (7, 8) derart sind, daß die durch diese zugeführte Stoffdichte so hoch ist, daß in einem Staukanal der Zwischenstoffauflaufkästen (7, 8) oder nachdem der Stoff von jeder Stauvorrichtung der Zwischenstoffauflaufkästen abgelassen ist, die bildenden Pulpeschichten einen solchen Filzgrad erreichen, daß sich die Fasern der Pulpe auf dem Drahtnetz (1) gegeneinander nicht nennenswert bewegen können, und daß die Entwässerung der Schichten hoher Stoffdichte entlang des Drahtnetzes stattfindet; und wobei ein einzelnes Drahtnetz (1) als Unterlage für die übereinanderliegenden Schichten vorgesehen ist, und wobei eine Druckrolle (9) zwischen den beiden Zwischenstoffauflaufkästen (7, 8) hoher Stoffdichte vorgesehen ist, um die zwischen den Stoffauflaufkästen (7, 8) gebildete Pulpeschicht zu glätten.
